

1

3,775,325

## PREPARATION OF SYNTHETIC HYDROCARBON LUBRICATING COMPOSITIONS

Oliver C. Kerfoot and Delmar D. Krehbiel, Ponca City, Okla., and George C. Feighner, Franklin Lakes, N.J., assignors to Continental Oil Company, Ponca City, Okla.

No Drawing. Filed May 30, 1972, Ser. No. 258,137

Int. Cl. C10m 1/16

U.S. Cl. 252—59

12 Claims 10

### ABSTRACT OF THE DISCLOSURE

Synthetic hydrocarbon lubricating compositions, such as those disclosed in U.S. Pat. 3,598,739, having improved pour point properties may be prepared in situ by Friedel-Crafts alkylation of a mixture of monoalkyl-substituted aromatic compounds containing at least 2 volume percent of tetrahydronaphthalene compounds with a halogenation product derived from partially chlorinating or brominating

5 the method of this invention, one can, in a single alkylation reaction, alkylate a mixture containing a relatively small quantity of tetrahydronaphthalene compounds in addition to the monoalkyl-substituted aromatic compounds and obtain a product composition of the general type disclosed in Sias.

The synthetic hydrocarbon lubricating compositions having improved pour point properties which may be prepared in accordance with the method of this invention include those described by Sias and may generally be described as comprising polyalkyl-substituted aromatic compounds of the formula

Ar(R)<sub>n</sub>

15 wherein Ar is benzene, toluene, or xylene; R is, independently, an alkyl group having 6 to 24 carbon atoms; and n is an integer of 2 or 3;

and at least 10 percent by volume, based on the polyalkyl-substituted aromatic compounds, of higher alkyl-substituted tetrahydronaphthalene compounds of the formula



wherein A is, independently, an alkyl group having 1 to 20 carbon atoms provided that when more than one A substituent is present the sum of carbon atoms for all A substituents is 2 to 20; y is 0 or an integer of 1—4; R' is independently, H or an alkyl group having 1 to 22 carbon atoms provided that the sum of carbon atoms for both R' substituents is 5 to 23; and x is an integer of 1—3.

In the above-described polyalkyl-substituted aromatic compounds, it is preferred that Ar is benzene; each R, independently, is a straight or branch chain C<sub>8</sub>—C<sub>20</sub> alkyl group, preferably C<sub>10</sub>—C<sub>18</sub>; and n is equal to 2.

In the above-described higher alkyl-substituted tetrahydronaphthalene compounds, it is preferred that each A, independently, is a straight or branch chain alkyl group having 1 to 13 carbon atoms provided that when both A substituents are alkyl groups the sum of carbon atoms is 6 to 14; y is equal to 2; each R' is, independently, H or a straight or branch chain alkyl group having 1 to 18 carbon atoms, preferably 1 to 16 carbon atoms, with the sum of both R' substituents being 7 to 19 carbon atoms, preferably 9 to 17; and x is equal to 1.

It has been found in accordance with the method of this invention that the above compositions may be prepared in a single step alkylation reaction as described hereinafter.

The material to be alkylated in forming compositions as described above is a mixture of monoalkyl-substituted aromatic compounds of the formula

ArR

60 and at least 2 percent by volume, based on the monoalkyl-substituted aromatic compounds, of tetrahydronaphthalene compounds of the formula



65 Ar, R, A and y are, in their broad and preferred forms, as defined above in connection with the polyalkyl-substituted aromatic compounds and the higher alkyl-substituted tetrahydronaphthalene compounds, respectively.

2

For convenience in describing the invention hereinafter, the above-described polyalkyl- and monoalkyl-substituted aromatic compounds will be referred to as PAA and MAA, respectively, and in their preferred forms when Ar is benzene and  $n$  is 2 they will be referred to as DAB and MAB, respectively. Similarly, the above-described higher alkyl-substituted tetrahydronaphthalene compounds and reactant tetrahydronaphthalene compounds in their broad sense will be referred to as HATHN and THN, respectively, and in their preferred forms wherein  $y$  is 2 and  $x$  is 1, they will be referred to as TTHN and DTHN, respectively.

As indicated above the mixture to be alkylated in accordance with the method of this invention comprises MAA containing at least 2 percent by weight, based on the MAA, of THN. It has unexpectedly been found that when such a mixture is alkylated as hereinafter described the resulting product composition contains at least 10 percent by volume, based on PAA, of HATHN. In general, it may be said that when the mixture being alkylated contains of the order of 20 volume percent THN, based on MAA, the resulting product composition will contain in excess of about 50 volume percent HATHN, based on PAA. It is contemplated that the mixtures being alkylated contain from about 2 volume percent up to about 30 volume percent THN, based on MAA, although it should be understood that greater amounts may be included and the upper limit of 30 volume percent does not form an essential feature of the invention. On the other hand, it is essential that the mixture contain at least about 2 volume percent of THN in order that the product composition contains sufficient HATHN to obtain the advantages discussed in the aforementioned Sias patent. For most product compositions intended for lubricant utility, the mixture being alkylated should preferably contain about 2 volume percent to 15 volume percent THN.

The MAA may be obtained by simple alkylation of an aromatic compound such as benzene, toluene or xylene, with an olefin or a chlorinated paraffin having the appropriate carbon content as is well-known in the art; for example, see the techniques described in U.S. 3,173,965. A particularly suitable technique for preparing MAA is also described in U.S. 3,316,294 wherein chlorinated paraffins are employed. In this latter process, some THN is also produced along with the MAA and thus provides a convenient source for the mixture to be alkylated in this invention, at least insofar as lesser quantities of THN may be required in the material to be alkylated. On the other hand, THN may be obtained by careful fractionation of the product prepared by the process described in U.S. 3,316,294 and thereafter added to the MAA in any proportion desired depending upon the mixture desired for the alkylation.

The halogenation product used to alkylate the mixture of MAA and THN may be derived by partially chlorinating or brominating  $C_6$ - $C_{24}$  paraffins to the extent whereby from about 10 to 35 mol percent of the paraffins become halogenated. The degree of halogenation should not exceed about 35 mol percent so as to attain satisfactory selectivity to the monohalogenated derivatives. On the other hand, the halogenation should exceed about 10 mol percent for practical reasons. While both bromine and chlorine may be employed as the halogenating agents, it is preferred to use chlorine due to its ready availability. Conventional halogenation techniques may be employed including both liquid or vapor phase conditions. A highly suitable halogenation technique which may be used to obtain suitable halogenation products useful in the method of this invention is described in U.S. 3,316,294, it being understood that the technique described therein is applicable with both branched and straight chain paraffins having 6 to 24 carbon atoms. Preferably, the halogenation product is derived from

straight chain paraffins having 8 to 20 carbon atoms, more preferably 10 to 18 carbon atoms. It is also pointed out that the partially halogenated reaction mixture may be employed as such in the method of this invention as the unreacted paraffins will merely be carried through the process as inert materials. Alternatively, the halogenated paraffins may be separated from the unreacted paraffins thus avoiding accommodation of the inerts in the process.

10 The alkylation reaction is preferably conducted as a Friedel-Crafts reaction using a suitably inorganic halide Friedel-Crafts catalyst such as  $AlCl_3$ ,  $AlBr_3$ ,  $FeCl_3$ ,  $SnCl_4$ ,  $BF_3$ ,  $BCl_3$ ,  $ZnCl_2$ ,  $HF$ ,  $H_2SO_4$ ,  $P_2O_5$ ,  $H_3PO_4$ , antimony chlorides, and mercuric chlorides. Preferably, the Friedel-Crafts catalyst is aluminum chloride or aluminum bromide with the most preferred catalyst being aluminum chloride.

15 The reaction may be carried out at temperatures in the range of about  $20^\circ$  to  $100^\circ$  C., preferably  $50^\circ$  to  $90^\circ$  C., using a molar ratio of MAA to the halogenated paraffin in the range of about 1:1 to about 10:1, preferably about 2:1 up to about 6:1. The quantity of catalyst which may be used may range from about 1 to about 10 percent by weight, based on the halogenated paraffin, preferably about 3 percent to about 8 percent by weight.

20 The alkylation reaction can be carried out in a continuous or batch-wise manner for a period of time sufficient to complete the alkylation as is well-known in the art. Thereafter, the reaction product effluent can be introduced into a separator whereupon a product phase and catalyst sludge phase are formed. The catalyst sludge phase may be easily decanted off and either removed from the process or recycled back to the alkylation reaction. The product phase may then be treated to remove 25 any acidic components by any conventional technique such as treating with sulfonic acid and washing with a caustic solution or percolation through a bauxite bed. After any such preliminary treatment, the product phase may be fractionally distilled to remove any unwanted lower boiling materials as desired.

30 The following examples are presented for the purposes of further illustrating the above-described method of this invention:

#### EXAMPLE 1

45 To a creased three-necked stirred flask, there were added 540 g of a mixture of linear tridecylbenzene ( $C_{13}$  MAB) containing 3.4 volume percent  $C_{13}$  tetrahydronaphthalenes (DTHN) and 150 g. of chlorinated  $C_{13}$  normal paraffin, and the flask was heated to about  $65^\circ$  C. 50 The chlorinated  $C_{13}$  normal paraffin was obtained by chlorinating a quantity of  $C_{13}$  normal paraffin to the extent of about 20 mol percent in accordance with the technique described in U.S. Pat. 3,316,294 followed by separation by distillation of any unreacted normal paraffin.

55 The  $C_{13}$  tetrahydronaphthalenes were obtained in admixture with tridecylbenzene by alkylating benzene with a partially chlorinated  $C_{13}$  paraffin also described in U.S. Pat. 3,316,294. Six g. of  $AlCl_3$  catalyst were then added and the mixture stirred for about  $1\frac{1}{2}$  hours while maintaining the temperature at about  $65^\circ$  C. The reaction mixture was then gravity settled into the two phases, an upper product phase and a lower catalyst sludge layer. The lower catalyst sludge layer (about 18 g.) was then removed while the remaining upper product phase was washed with

60 dilute aqueous caustic and distilled to remove the lower boiling unreacted materials with the cut being taken at  $220^\circ$  C. a 10 millimeters Hg. The resulting 219 g. of product, by mass spectrometer analysis, comprises  $C_{13}$  dialkylbenzene (DAB) containing about 14 volume percent higher alkyl tetrahydronaphthalenes (TTHN).

#### EXAMPLE 2

65 For comparison, the procedure set forth in Example 1 was repeated except that the starting tridecylbenzene 75 ( $C_{13}$  MAB) contained no  $C_{13}$  tetrahydronaphthalenes

(DTHN) as taught in the prior art. The resulting dialkylbenzene product amounted to 170 g. of which mass spectrometer analysis indicated that only 3 volume percent of higher alkyl tetrahydronaphthalenes (TTHN) were present.

## EXAMPLE 3

In a further example of the method of this invention, 1400 g. of a mixture of MAB ( $C_{12}$ – $C_{14}$  monoalkylbenzenes) containing 6.4 volume percent DTHN ( $C_{12}$ – $C_{14}$  tetrahydronaphthalenes), 1170 g. of partially chlorinated  $C_{12}$ – $C_{14}$  normal paraffins were charged to a creased three-necked stirred flask and heated to about 70° C. The mixture of MAB and DTHN was prepared in accordance with the technique described in U.S. Pat. 3,316,294. The partially chlorinated paraffins were prepared as described in the same patent, the extent of chlorination being approximately 20 mol percent. 18  $AlCl_3$  catalyst were then added to the flask and the reaction mixture was stirred at 70° C. for about 1½ hours. The reaction mixture was then gravity settled into two phases and the lower catalyst sludge layer (about .58 g.) was removed. The remaining product mixture was washed with a dilute aqueous caustic solution and distilled to remove the lower boiling unreacted materials with the cut point being taken at 225° C. and 10 millimeters Hg. The DAB product mixture amounting to about 484 g. was found to contain, by mass spectrometer analysis, 78 volume percent dialkylbenzenes (DAB) and 19.2 volume percent higher alkyl tetrahydronaphthalenes (TTHN). In addition, the unreacted MAB fraction recovered from the distillation step was found by mass spectrometer analysis to contain 5.8 volume percent of the DTHN.

The DAB product mixture possessed very attractive low temperature physical properties as outlined in Table 1 hereinafter.

## EXAMPLE 4

In a further example demonstrating the method of this invention, the unreacted MAB fraction recovered from the distillation step in Example 3 was subjected to alkylation as follows: 850 g. of the recovered MAB fraction containing 5.8 volume percent of  $C_{12}$ – $C_{14}$  tetrahydronaphthalenes (DTHN) was charged to a three-necked stirred flask along with 527 g. of partially chlorinated  $C_{12}$ – $C_{14}$  normal paraffins as described in Example 3, and the mixture was heated to about 70° C. Seven g. of  $AlCl_3$  catalyst were then added to the flask and the reaction mixture was stirred for about 1½ hours at 70° C. Thereafter, the reaction mixture was gravity settled into two phases at the lower catalyst sludge layer, amounting to about 28 g. was removed. The remaining product mixture was then washed with a dilute aqueous caustic solution and distilled to remove the lower boiling unreacted materials with the cut point being taken at 225° C. and 10 millimeters Hg. The resulting dialkylbenzene (DAB) product mixture amounted to about 236 g. and contained by mass spectrometer analysis about 23 volume percent higher alkyl tetrahydronaphthalenes (TTHN). The product again exhibited good low temperature physical properties which are outlined in the following table.

TABLE 1

| Example 3         | 3      | 4      |
|-------------------|--------|--------|
| Viscosity, cs. at |        |        |
| –40° F.           | 11,669 | 11,082 |
| +100° F.          | 33.5   | 33.2   |
| +210° F.          | 5.8    | 5.5    |
| Viscosity index   | 115    | 114    |
| Pour point, ° F.  | –65    | –65    |

Thus, having described the invention in detail, it will be understood by those skilled in the art that certain modifications and variations may be made in the invention without departing from the spirit and scope thereof as defined herein and in the appended claims.

We claim:

1. A method of preparing a synthetic hydrocarbon lubricating composition comprising polyalkyl-substituted aromatic compounds of the formula



wherein Ar is benzene, toluene, or xylene; R is, independently, an alkyl group having 6 to 24 carbon atoms; and n is an integer of 2 or 3; and at least 10% by weight, based on the polyalkyl-substituted aromatic compounds, or higher alkyl-substituted tetrahydronaphthalene compounds of the formula



wherein A is, independently, an alkyl group having 1 to 20 carbon atoms provided that when more than one A substituent is present the total number of carbon atoms for all A substituents is 2 to 20; y is 0 or an integer of 1–4; R' is, independently, H or an alkyl group having 1 to 22 carbon atoms provided that the total number of carbon atoms for both R' and substituents is 5 to 23; x is an integer of 1–3;

which method comprises alkylating a mixture containing monoalkyl-substituted aromatic compounds of the formula  $Ar(R)$ , both Ar and R being as defined above, and at least 2% by weight, based on the monoalkyl aromatic compounds, of tetrahydronaphthalene compounds having the formula



both A and y being as defined above, in a Friedel-Crafts reaction with a halogenation product derived from partially chlorinating or brominating  $C_6$  to  $C_{24}$  paraffins to the extent whereby from about 10 to 35 mol percent of the paraffins are halogenated.

2. A method according to claim 1 wherein the mixture being alkylated contains about 2 volume percent to 30 volume percent of said tetrahydronaphthalene compounds.

3. A method according to claim 1 wherein in the monoalkyl-substituted aromatic compounds, Ar is benzene and R is a straight or branched chain  $C_8$ – $C_{20}$  alkyl group.

4. A method according to claim 3 wherein R is a straight or branched chain  $C_{10}$ – $C_{18}$  alkyl group.

5. A method according to claim 3 wherein R is a straight chain alkyl group.

6. A method according to claim 3 wherein in tetrahydronaphthalene compounds, A is a straight or branched chain alkyl group having 1 to 13 carbon atoms and y is equal to 2.

7. A method according to claim 6 wherein the alkyl group represented by A is straight chain.

8. A method according to claim 6 wherein the mixture being alkylated contains about 2 volume percent to about 15 volume percent of said tetrahydronaphthalene compounds.

9. A method according to claim 1 wherein the alkylation is carried out at temperatures in the range of about 20° to 100° C. in the presence of a Friedel-Crafts catalyst.

10. A method according to claim 9 wherein the halogenation product is derived from partially chlorinating  $C_6$ – $C_{20}$  paraffins.

11. A method according to claim 10 wherein the molar ratio of monoalkyl-substituted aromatic compounds to halogenated paraffins is in the range of about 1:1 to about 10:1.

12. A method according to claim 9 wherein the quantity of catalyst used is in the range of about 1 to 10 weight percent based on the halogenated paraffins.

|           |        |                       |            |
|-----------|--------|-----------------------|------------|
| 3,391,210 | 7/1968 | Feighner et al. ----- | 260—671 BX |
| 3,598,739 | 8/1971 | Sias -----            | 260—59     |
| 3,661,780 | 5/1972 | Feighner et al. ----- | 260—59     |

**References Cited**  
**UNITED STATES PATENTS**

|           |         |                       |            |
|-----------|---------|-----------------------|------------|
| 3,538,178 | 11/1970 | Sias -----            | 252—59 X   |
| 3,662,012 | 5/1972  | Feighner et al. ----- | 260—672 T  |
| 3,458,447 | 7/1969  | Shultz -----          | 260—671 BX |

5 DANIEL E. WYMAN, Primary Examiner  
 W. H. CANNON, Assistant Examiner

U.S. Cl. X.R.  
 260—671 B